

## UNITED STATES PATENT OFFICE.

JAKOB SCHWARZKOPF, OF ELMSHORN IN HOLSTEIN, GERMANY.

## POLISHING COMPOSITION.

No Drawing. Application filed March 23, 1925, Serial No. 17,800, and in Germany January 21, 1925.

In the production of oil of roses from roses a wax-like substance is obtained as a by-product, which is sold as rose-wax. In the course of experiments for the utilization of rose-wax for industrial purposes it was found that rose-wax acts similarly to coffee-wax in polishing compositions for leather, linoleum, wood and the like as a means for increasing the brilliancy of the polish. Hence, rose-wax can be utilized in the polishing compositions as a substitute for coffee-wax. As compared with coffee-wax it has certain advantages:—

- (1) It reduces the volatilization of the wax solvent in the polishing compositions.
- (2) An addition of rose-wax increases the polish on the surface in the container.

A suitable proportion of coffee-wax and rose-wax in polishing compositions is, for instance, 50 parts coffee-wax, 50 parts rose-wax. It is, however, also possible to use a smaller addition of rose-wax and the coffee-wax may be entirely replaced by rose-wax.

The constituents of the polishing composition may, for instance, be used in the following proportions by weight:—

|                                                    | Parts. |
|----------------------------------------------------|--------|
| Montan wax                                         | 7      |
| Carnauba wax                                       | 5      |
| 20 Ceresine                                        | 16     |
| Aniline dyes                                       | 4      |
| Oil of turpentine                                  | 68     |
| A mixture of coffee-wax and rose-wax half-and-half | 1-3    |

Rose wax, like coffee wax, not only increases the brilliancy but has the characteristic property not possessed by any other wax of imparting to the polishing agent special homogeneity and permits very fine sub-division of the polishing agent. Due to the great economy in the use of the polishing agent greater brilliancy is obtained.

Having now particularly described and ascertained the nature of my said invention and in what manner the same is to be performed, I declare that what I claim is:—

1. A polishing composition of wax-like character for leather, linoleum, wood and the like containing as ingredients rose wax and coffee wax.

2. A polishing composition of wax-like character for leather, linoleum, wood and the like consisting of Montan and carnauba waxes, ceresine, aniline dyes, oil of turpentine, and a mixture of coffee wax and rose wax.

3. A polishing composition as claimed in claim 2 characterized in that the ingredients are combined in the following proportions by weight: Montan wax 7 parts, carnauba wax 5 parts, ceresine 16 parts, aniline dyes 4 parts, oil of turpentine 68 parts, and 1 to 3 parts of coffee-wax and rose-wax.

In testimony whereof I affix my signature.

JAKOB SCHWARZKOPF.